

# UNITED STATES PATENT OFFICE.

UGO ALVISI, OF ROME, ITALY.

## DETONATING COMPOUND.

SPECIFICATION forming part of Letters Patent No. 707,493, dated August 19, 1902.

Original application filed December 17, 1898, Serial No. 699,562. Divided and this application filed October 10, 1901. Serial No. 78,245. (No specimens.)

To all whom it may concern:

Be it known that I, UGO ALVISI, a subject of the King of Italy, residing at 12 Via Carlo Alberto, Rome, in the Kingdom of Italy, have 5 invented certain new and useful Improvements in Detonating Compounds, of which the following is a specification.

This invention relates to an improved detonating compound, as hereinafter described.

10 It is common practice to add to the fulminate of mercury, when such is employed for charging detonators, saltpeter or chlorates, and so on, for the purpose of obtaining different effects as may be desired for special requirements.

I have manufactured detonating materials specially for use in charging caps (detonators) by mixing perchlorate of ammonium to the fulminate of mercury. The mixture of 20 17.20 per cent. of perchlorate of ammonium with 83.80 of fulminate of mercury produces the maximum effect, and I have found it to be the most powerful of detonators, both as to its range of explosive force and its breaking power. It may be employed in all cases where ordinarily fulminate of mercury is used as a detonator—for example, for firing dynamite, nitroglycerin, nitrocellulose, picric acid, &c., When the explosive—dynamite, for example—itself contains perchlorate of ammonium, the charge of fulminate of mercury in the detonator may be reduced. Supposing we have dynamite of the following composition: nitroglycerin, seventy-five; soluble cotton, (collodion,) five; cellulose, five; perchlorate of ammonium, fifteen. The most convenient detonator for detonating the same is that which contains only sixty per cent. of fulminate of mercury and the rest perchlorate of ammonium.

In other cases—for example, with ordinary caps for shooting—the amount of the perchlorate may be increased by reducing that of the fulminate. Obviously to this mixture may be added other oxidizing and combustible substances, care being taken, however, to avoid potassium salts—for example, saltpeter, chlorate of potassium, (except perchlorate of potassium)—which would react with the perchlorate of ammonium and produce compounds which would either be unstable or deliquescent. These mixtures are prepared in the ordinary manner similar to that adopted, for example, for preparing mixtures of fulminate of mercury and chlorate of potassium, and the caps or detonators are charged therewith in the ordinary way. It is preferable to provide metallic caps with an internal lining to prevent the mixture from coming into contact with the metal. The detonators manufactured with these mixtures are employed like ordinary detonators, and they may be fired either by means of a tape-primer, percussion-fuse, or by the electric spark.

What I claim, and desire to secure by Letters Patent of the United States, is—

1. A detonating compound containing fulminate of mercury and perchlorate of ammonium.

2. A detonating compound containing 17.20 per cent. of perchlorate of ammonium and 83.80 per cent. of fulminate of mercury.

In testimony whereof I have hereunto set my hand, in presence of two subscribing witnesses, this 19th day of September, 1901.

UGO ALVISI.

Witnesses:

ING. C. PERRAN,  
RICHARD C. G. KLOSS.